

1

3,240,577

### MOTOR FUEL COMPOSITION

Alfred Arkell and George W. Eckert, Wappingers Falls, N.Y., assignors to Texaco Inc., New York, N.Y., a corporation of Delaware  
No Drawing. Filed May 25, 1962, Ser. No. 197,584  
13 Claims. (Cl. 44—69)

This invention relates to a motor fuel composition containing a novel anti-knock additive. More particularly, the invention relates to a motor fuel for spark ignition internal combustion engines containing a hydrocarbyl selenite anti-knock agent.

Present day internal combustion engines have high compression ratios and require high octane fuels for satisfactory performance. This places a severe strain on petroleum refiners to produce fuels having the necessary high octane ratings demanded by these engines. The trend to higher compression ratios is continuing and it is estimated that motor fuels having octane ratings of the order of 105 and above will be required in the foreseeable future.

At the present time, premium motor fuels having octane ratings of 97 or above are generally provided by relying heavily on refining operations, such as fluid catalytic cracking, catalytic reforming, alkylation and isomerization, in conjunction with the use of a conventional anti-knock additive, such as a tetraalkyl lead compound. Frequently, these steps are not satisfactory to efficiently or economically produce a high octane motor fuel. As a result, many proposals have been made directed to fuel compositions containing additional additives, such as octane appreciators and the like, to supplement the anti-knock property of present day premium motor fuels. Dialkyl selenides are among the materials that have been proposed as motor fuel additives. They were not sufficiently effective to be adopted commercially and also possessed an extremely objectionable odor. The hydrocarbyl selenites of the present invention are extremely effective anti-knock additives and are free of objectionable odors.

The subject invention involves the discovery that a gasoline or motor fuel can be substantially improved with respect to its anti-knock property by the addition of 0.01 to 5 volume percent of a hydrocarbyl selenite. Hydrocarbyl selenites are true anti-knock agents as evidenced by the fact that they will substantially improve the octane rating of a motor fuel in the absence of any other anti-knock additive.

This invention is characterized by a number of important features. It is surprising that hydrocarbyl selenites are anti-knock agents since similar hydrocarbyl esters of elements from the same subgroup of the periodic table, namely tellurium and sulfur, either are not readily prepared or impart a pro-knock effect to motor fuels. Another feature is that hydrocarbyl selenites impart a substantial anti-knock improvement to both very low and very high octane motor fuels. Still another important feature is that these compounds impart a substantial additional anti-knock improvement to leaded motor fuels, i.e., motor fuels previously improved in octane value by the presence of a conventional tetraalkyl lead anti-knock agent.

The hydrocarbyl selenite additives of this invention are represented by the following formula:



in which R and R' each represent a hydrocarbyl radical having from 1 to 18 carbon atoms. R and R' may each represent an alkyl, aryl, alkaryl, aralkyl or alicyclic hydrocarbyl radical and will generally have from 1 to 8

2

carbon atoms. Primary alkyl hydrocarbyl selenites and, in particular, primary branched-chain alkyl hydrocarbyl selenites are preferred with a specific preferred species being diisobutyl selenite. It has been theorized that the greater effectiveness of the primary alkyl hydrocarbyl selenites is due to the formation during engine operation of aldehydes, which have an octane appreciator effect on lead, if present, and to the selenium-containing residue formed on decomposition.

10 The anti-knock additives of this invention can be prepared by reacting the corresponding hydrocarbyl alcohol with selenium dioxide according to the following equation:



15 For example, two moles of isobutanol are reacted with a mole of selenium dioxide to produce diisobutyl selenite. This reaction takes place readily by azeotropic removal of water from a mixture of the alcohol and selenium dioxide.

20 The reaction proceeds at ambient pressures and at the normal boiling point of the azeotrope being formed. Diisobutyl selenite, isobutyl alcohol and water form an azeotrope consisting of 33% by weight of water which boils at 89.8° C. It should be noted that an excess of 25 the alcohol (over and above the 2 moles necessary for reaction) will be required for the azeotropic removal of water formed during the reaction. The required excess is 0.5 to 1.0 mole of alcohol per mole of water removed.

Typical hydrocarbyl selenites which can be employed 30 in this invention in addition to diisobutyl selenite include, diisoamyl selenite, dimethyl selenite, diethyl selenite, isobutyl propyl selenite, ethyl isopropyl selenite, di-2-ethylhexyl selenite, didodecyl selenite (so called dilauryl), dibenzyl selenite, di-n-propyl selenite, di-n-butyl selenite, 35 dioctadecyl selenite (so called distearyl), ditolyl selenite and the like.

The motor fuels of the invention consist of gasoline hydrocarbons and a minor amount sufficient to impart an improved anti-knock property to the fuel of a hydrocarbyl selenite having the formula set forth above in which each hydrocarbyl radical has from 1 to 18 carbon atoms. Generally, the hydrocarbyl selenite will amount to about 0.01 to 5 volume percent of the fuel with amounts between 0.1 and 2.5 volume percent being preferred. These fuels will generally contain aromatic and/or olefin components in addition to the paraffins ordinarily present in a motor fuel. The aromatic and/or olefin components can constitute as high as 100 volume percent of the fuel but usually will amount to between about 20 and 80 volume percent. There are no critical requirements with respect to the proportions of the volatile hydrocarbon component types in the fuel.

A valuable feature of this invention is that an organo-lead anti-knock agent can also be employed jointly with the hydrocarbyl selenite to produce a motor fuel composition having an unusually high octane rating. The organo-lead additives generally employed for anti-knock purposes in motor fuels are the tetraalkyl lead compounds. Typical tetraalkyl lead anti-knock compounds are tetraethyl lead, tetramethyl lead, tetrabutyl lead, tetraamyl lead, tetrapropyl lead, mixtures thereof and the like.

The tetraethyl lead mixture commercial available for automotive use contains an ethylene chloride-ethylene bromide mixture as a scavenger for removing lead from the combustion chamber in the form of volatile lead halides. This product comprises tetraethyl lead, ethylene chloride and ethylene bromide, the latter two reagents being present in 1.0 theory and 0.5 theory, respectively, theory denoting stoichiometric amount required for reaction with the lead content of the tetraethyl lead.

70 The organo-lead reagent is employed in motor fuel compositions in concentrations between 0.5 ml. per gal-

Ion up to the statutory limit of organo-lead reagent concentration, which at the present time is 4 ml. per gallon for automotive fuel. The usual concentration of the tetraethyl lead is between 1 and 3 ml. per gallon in gasoline.

The improvement in motor fuels containing fuels containing a hydrocarbyl selenite of the invention was demonstrated by incorporating measured amounts of diisobutyl selenite in various fuel compositions and determining the incremental increase in their R.O.N. (Research Octane Number). In these runs, diisobutyl selenite was employed as the sole anti-knock agent, i.e., in the absence of any conventional anti-knock agent. Four fuels representing both high and low octane fuels were employed in this test. Test Fuel A was substantially pure isoctane having an R.O.N. of 100.0. Test Fuel B was an alkylate fuel boiling from 126° F. to 368° F. and having an R.O.N. of 97.5. Test Fuel C was a heavy straight run naphtha having an R.O.N. of 52.0, and Test Fuel D was a platformate boiling from 130° F. to 394° F. having an R.O.N. of 91.2. Various amounts of diisobutyl selenite were incorporated into these fuels and the incremental increase in R.O.N. value determined. These results of these tests are tabulated in Table I below.

TABLE I  
*Octane effect of diisobutyl selenite in unleaded fuels*

|        | Diisobutyl Selenite, Percent vol. | Research Δ R.O.N. |
|--------|-----------------------------------|-------------------|
| Fuel A | 0.5                               | 3.2               |
| Do     | 1.0                               | 5.4               |
| Do     | 2.0                               | 7.4               |
| Fuel B | 0.5                               | 1.7               |
| Do     | 1.0                               | 4.2               |
| Do     | 2.0                               | 8.5               |
| Fuel C | 0.5                               | 1.6               |
| Do     | 1.0                               | 6.0               |
| Do     | 2.0                               | 14.0              |
| Fuel D | 0.5                               | 2.8               |
| Do     | 1.0                               | 5.2               |

The improvement in leaded motor fuels, i.e., motor fuels containing 3 cc. per gallon of tetraethyl lead fluid, brought about by the addition of a hydrocarbyl selenite was demonstrated by incorporating measured amounts of diisobutyl selenite into various motor fuels and then determining the incremental increase in their R.O.N. values as above. Three leaded fuels having different octane values were employed in these tests. Test Fuel E was a regular grade gasoline boiling from 104° F. to 418° F. and having an R.O.N. value of 94.0. Test Fuel F was a premium grade motor fuel boiling from 91° F. to 370° F. and having an R.O.N. of 99.4 and Test Fuel G was a super premium grade motor fuel boiling from 88° F. to 370° F. and having an R.O.N. of 106.0. The incremental R.O.N. improvement in these leaded fuels brought about by adding diisobutyl selenite is shown in Table II below.

TABLE II  
*Octane effect of diisobutyl selenite in leaded fuels*

|        | Diisobutyl Selenite, Percent vol. | Research Δ R.O.N. |
|--------|-----------------------------------|-------------------|
| Fuel E | 0.5                               | 1.4               |
| Do     | 0.75                              | 2.4               |
| Do     | 1.00                              | 3.4               |
| Do     | 1.50                              | 5.5               |
| Fuel F | 0.75                              | 1.1               |
| Do     | 1.00                              | 1.9               |
| Do     | 1.5                               | 4.9               |
| Do     | 2.0                               | 6.0               |
| Do     | 2.5                               | 7.0               |
| Fuel G | 0.75                              | 2.3               |
| Do     | 1.00                              | 3.6               |
| Do     | 1.5                               | 4.5               |
| Do     | 2.0                               | 5.1               |

The data in the table below shows the improved anti-

knock effect of dimethyl selenite in an unleaded motor fuel. This gasoline, designated Fuel H, boiled in the range of 96° F. to 374° and had a R.O.N. of 94.7.

TABLE III

|           | Diisobutyl Selenite, Percent vol. | Research Δ R.O.N. |
|-----------|-----------------------------------|-------------------|
| 10 Fuel H | 0.5                               | 4.7               |
| Do        | 1.0                               | 6.0               |
| Do        | 2.0                               | 7.9               |

The foregoing data demonstrate the effectiveness of hydrocarbyl selenites as true anti-knock agents in a variety of leaded and unleaded motor fuel compositions. These data also show that motor fuels of unusually high octane value may be obtained through the use of the additive of the invention.

We claim:

1. A hydrocarbon fuel in the gasoline boiling range containing an effective anti-knock amount of a hydrocarbyl selenite having the formula:



in which R and R' each represent a hydrocarbyl radical having from 1 to 18 carbon atoms.

2. A fuel according to claim 1 in which said hydrocarbyl selenite amounts to about 0.01 to 5 volume percent of said fuel.

3. A fuel according to claim 1 in which R and R' each represent a primary alkyl radical having from 1 to 8 carbon atoms.

4. A hydrocarbon fuel in the gasoline boiling range containing an effective anti-knock amount of diisobutyl selenite.

5. A hydrocarbon fuel in the gasoline boiling range containing an effective anti-knock amount of dimethyl selenite.

6. A hydrocarbon fuel according to claim 4 in which said diisobutyl selenite amounts to 0.1 to 2.5 volume percent.

7. A hydrocarbon fuel according to claim 5 in which said dimethyl selenite amounts to 0.1 to 2.5 volume percent.

8. A motor fuel in the gasoline boiling range containing an effective anti-knock amount of a tetraalkyl-lead compound and a hydrocarbyl selenite having the formula:



in which R and R' each represent a hydrocarbyl radical having from 1 to 18 carbon atoms.

9. A motor fuel according to claim 8 in which said organo-lead compound amounts to 0.5 to 3.0 ml. per gallon and said hydrocarbyl selenite amounts to 0.01 to 5 volume percent of said fuel.

10. A motor fuel according to claim 8 in which said organo-lead compound is a tetra-alkyl lead compound.

11. A motor fuel according to claim 10 in which R and R' in said hydrocarbyl selenite each represent a primary alkyl radical having from 1 to 8 carbon atoms.

12. A motor fuel according to claim 10 in which said hydrocarbyl selenite is diisobutyl selenite.

13. A motor fuel according to claim 10 in which said hydrocarbyl selenite is dimethyl selenite.

References Cited by the Examiner

UNITED STATES PATENTS

1,575,436 3/1926 Midgley ----- 44-76

(Other references on following page)

## UNITED STATES PATENTS

|           |        |                         |       |
|-----------|--------|-------------------------|-------|
| 1,906,724 | 5/1933 | Rosenstein et al. ----- | 44-76 |
| 1,920,766 | 8/1933 | Rosenstein et al. ----- | 44-76 |
| 2,151,432 | 3/1939 | Lyons et al. -----      | 44-69 |
| 2,460,700 | 2/1949 | Lyons et al. -----      | 44-68 |

## FOREIGN PATENTS

33,371 6/1924 Denmark.

## OTHER REFERENCES

Organic Chemistry, by Richter, 2nd edition, 1919, page 148.

“The Effect of Metallic Vapours on the Ignition of Substances,” Journal of Institution of Petroleum Technologists, February-December 1927, vol. 13, pages 244-255.

DANIEL E. WYMAN, *Primary Examiner.*